

## UNITED STATES PATENT OFFICE

CHARLES P. TEEPLE, OF CHICAGO, ILLINOIS, ASSIGNOR TO CRANE PACKING COMPANY, OF CHICAGO, ILLINOIS, A CORPORATION OF ILLINOIS

## LUBRICANT

No Drawing.

Application filed October 29, 1930. Serial No. 492,093.

My invention relates to a lubricant particularly adapted for use in engines, pumps, machinery, etc., for lubricating parts in situations in which the lubricant is more or less exposed to contact with gasoline or other petroleum fuel. The ordinary lubricants on the market are more or less soluble in petroleum products and are, therefore, not well adapted for use in such situations as they quickly become diluted or are dissolved out of the bearing which they are intended to protect. The object achieved by my invention is the production of a lubricant which will remain substantially insoluble and unattacked in contact with gasoline or the like. My improved lubricant has the further advantage of not being readily soluble in water so that it is not materially affected by any water, which may be carried by the gasoline or other petroleum products or by water from an outside source, to which the lubricant is exposed.

In its preferred composition my lubricant comprises the following ingredients: blown castor oil, glycerine, carnauba wax and graphite to which may be added a small amount of fragrant material such as oil of sassafras, nitrobenzine, eucalyptus or acacia to improve the odor.

These ingredients may be mixed in varying proportions, depending upon the consistency and other properties desired, but as a specific example of a composition which I have found satisfactory for general service may be given the following:

|                           | Per cent<br>by weight |
|---------------------------|-----------------------|
| Blown castor oil          | 53.0                  |
| Glycerine                 | 28.7                  |
| Carnauba wax No. 2        | 2.7                   |
| Graphite, dry, fine flake | 15.3                  |
| Oil of sassafras          | 0.3                   |

For satisfactory results it is necessary that the castor oil be blown more or less in order to reduce its solubility to the desired point, though the amount of blowing may vary somewhat according to the properties which it is desired that the lubricant shall have. The blowing also increases the viscosity of the oil. In the specific example given above the castor oil, which was of the ordinary type,

was blown by passing air therethrough while the oil was maintained at a temperature between 75° and 150° C. until the oil had a viscosity of about 25700 Saybolt universal at 100° F. In preparing the mixture the given quantity of blown oil and glycerine were dumped into a mixer equipped with steam coils and provided with an adequate stirring device of paddle type. When the mixture reached a temperature of 85° C., the above given quantity of carnauba wax was melted and poured into the mixture. The heat was then turned off and the agitation continued. After the ingredients mentioned had been thoroughly mixed the given amount of graphite was added. After the mixture had cooled to a thin, paste-like consistency the oil of sassafras was added and thoroughly mixed in. The lubricant was then ready to be poured into the receptacle for storage and use.

While the above mixture is very satisfactory for general purposes, the proportions given are not essential, but may vary within wide limits, depending upon the viscosity and other properties which it is desired that the lubricant shall have. It is not necessary to employ oil of sassafras or, indeed, any fragrant material. By varying the amount of carnauba wax, glycerine and blown castor oil, the viscosity of the composition may be varied as desired. Other waxes, as for example, Montan or Candelilla may be employed in place of carnauba wax or, if a thinner lubricant is desired the wax may be omitted altogether. The amount of graphite may also be varied within wide limits.

I have found that compositions within the following limits are suitable for my improved lubricant, as above stated, depending upon the particular properties desired or the purpose to which the lubricant is to be put:

|                      |        |
|----------------------|--------|
| Blown castor oil     | 25-80% |
| Glycerine            | 10-65% |
| Carnauba wax         | 0-25%  |
| Graphite or plumbago | 0-40%  |

My invention provides a lubricant which is substantially insoluble in gasoline or other petroleum products and may be used to ad-

vantage in packings, bearings or elsewhere in situations where the lubricant is exposed to the action of gasoline or the like with no substantial depreciation or loss by reason of being dissolved out. Furthermore, the lubricant resists the action of water to which it may be exposed whether the water be contained in the gasoline or other petroleum products in contact with the lubricant or is 10 from an outside source.

I claim:

1. A lubricant for gasoline pumps, etc., comprising 25 to 80% of blown castor oil and 10 to 65% glycerine.
- 15 2. A lubricant for gasoline pumps, etc., comprising blown castor oil, glycerine and graphite.
3. A lubricant for gasoline pumps, etc., comprising blown castor oil 25 to 80 per cent, glycerine 10 to 65 per cent and graphite 1 to 20 40 per cent.
4. A lubricant for gasoline pumps and the like comprising blown castor oil, glycerine and wax.
- 25 5. A lubricant for gasoline pumps, etc., comprising blown castor oil 25 to 80 per cent, glycerine 10 to 65 per cent and wax 1 to 25 per cent.
6. A lubricant for gasoline pumps, etc., comprising blown castor oil, glycerine, wax 30 and graphite.
7. A lubricant for gasoline pumps, etc., comprising blown castor oil 25 to 80 per cent, glycerine 10 to 65 per cent, wax 1 to 25 per 35 cent and graphite 1 to 40 per cent.
8. A lubricant for gasoline pumps, etc., having the following composition: blown castor oil about 53 per cent, glycerine about 28.7 per cent, carnauba wax about 2.7 per 40 cent, graphite about 15.3 per cent.

In testimony whereof, I have subscribed my name.

CHARLES P. TEEPLE.